

May 7, 1946.

C. H. WARD

2,399,964

METHOD OF ELECTRO-GALVANIZING

Original Filed March 11, 1940

2 Sheets-Sheet 1

Fig. 1.



May 7, 1946.

C. H. WARD

2,399,964

## METHOD OF ELECTRO-GALVANIZING

Original Filed March 11, 1940 2 Sheets-Sheet 2



Inventor

*Clemson H. Ward.*  
By *R. S. C. Mougherly*

Attorney

## UNITED STATES PATENT OFFICE

2,399,964

## METHOD OF ELECTROGALVANIZING

Clemson H. Ward, Baltimore, Md., assignor to  
Bethlehem Steel Company, a corporation of  
Pennsylvania

Original application March 11, 1940, Serial No.  
323,300. Divided and this application May 16,  
1942, Serial No. 443,264

7 Claims. (Cl. 204—28)

This invention relates to a method for treating flat rolled metal products, sheets, strip or plates in one or more liquid baths in which said flat rolled products disposed in a vertical plane are passed horizontally through cells or tanks containing the treating liquid, and is a division of my copending applications Serial Nos. 323,300 and 383,135, filed March 11, 1940, and March 6, 1941, respectively. The former has matured into Patent No. 2,384,660 of September 11, 1945.

In particular the invention relates to a method for electroplating flat rolled products in which said products are passed, without deviating from a vertical plane, through a succession of cells or enclosures in which cleaning, electroplating, slightly deplating, rinsing, drying and other operations are performed upon same.

One of the objects of my invention relates to the method of coating a sheet of metal with zinc by electrodeposition, which comprises subjecting the sheet as an anode to the action of an electric current in the presence of an electrolyte to clean the sheet, then subjecting the sheet as a cathode in the presence of an electrolyte for zinc plating in a cell or a plurality of cells each having an individual electric circuit connection on each side of each cell, and finally subjecting the plated sheet as an anode to the action of an electric current in the presence of an electrolyte to slightly deplate the coating on the sheet.

This electrolyte consists of an aqueous solution of zinc sulphate and sulphuric acid.

Another object of my invention relates to the method of treating the coating after the plating operation to produce a uniform bright finish or polished surface.

Other objects will appear hereinafter.

Having thus given a general description of the objects of my invention, I will now in order to make the same more clear, refer to the annexed two sheets of drawings forming a part of this specification and in which like characters of reference indicate like parts.

Figure 1 is a diagrammatic view in side elevation of my improved galvanizing plant illustrating the general arrangement of the complete apparatus for plating sheets; and

Figs. 2 and 3 show longitudinal transverse sections of the feeding in and discharge ends of the plant, respectively, taken on the line 3—3 of Fig. 1.

Referring now to the various characters of reference on the drawings, the numeral 1 designates the base member having a strip of insulation 2 thereon upon which the cells and roll boxes are

mounted and assembled together in longitudinal alignment above the launder 3 extending under the apparatus for receiving the waste water discharged therefrom. Adjacent to the launder 3 and on the same level are the launders 4 and 5 for receiving the electrolytes from the plating and first anodic cell 12, respectively, from which each are returned to a sump (not shown) where it is cooled and the electrolytes recirculated.

10 The sheet 6 to be plated is disposed in a vertical position between pairs of side rods 7, with its lower edge engaging grooved rollers 8, of a feed table 9, and advanced manually, or in any approved manner into the electrolytic galvanizing plant from the right hand end of the apparatus as indicated in Figure 1, where it first passes between a pair of contact rolls 10 in the roll box 11 then into the pickling bath in the anodic cell 12, where the surface of the sheet is thoroughly cleaned and freed from rust, scale, oil, grease, etc. In the anodic cell 12 the polarity of the electric circuit is reversed to that of the plating cells and the sheet forms the anode, and the lead inner lining of the cell the cathode as it passes through 15 the path in this cell. The sheet is then advanced between a pair of rubber-covered squeegee or sealing rolls 13 in roll box 14 and then is advanced between another pair of squeegee rolls 15 in the roll box 16, which guides the advancing end of the sheet into the first of a series of plating cells, of which seven are shown for illustration numbered 17, 18, 19, 20, 21, 22 and 23, but a greater or less number of plating cells may be used if desired. As shown in Figure 1, each plating cell has 20 at its left hand end a contact roll box indicated as 24, 25, 26, 27, 28, 29 and 30, respectively in each of which is mounted a pair of lead covered contact rolls 31, between which the sheet being plated is passed. After passing through the plating cells and between the pairs of contact rolls in sequence it is then fed into an anodic cell 32 and between a pair of contact rolls 33 in roll box 34 in which 25 the polarity of the electric circuit is reversed to that of the plating cells. In this case the sheet would again form the anode and the lead lining of the cell the cathode, the positive side 35 of the circuit extending to the contact rolls and the negative side of the circuit 36 to the side of the cell. In this manner the surface of the coating is slightly deplated thereby producing a uniformly bright finish or polished surface. After passing through the anodic cell 32 and between the contact rolls 33 in roll box 34 it is then fed into roll box 37 between a pair of squeegee rolls 38 which 30 retain the electrolyte in the roll box 34 and then

advanced between another pair of squeegee rolls 39 in roll box 48, thence into a wash box 41 having perforated pipes 42 for spraying water on each side of the sheet then into a drying box 43 having perforated steam pipes 44 for heating the sheet and finally the sheet passes between another pair of squeegee rolls 46 in a roll box 46 for wiping the surface of the sheet, from which point it is ejected onto a receiving table 47 which is constructed in a similar manner as the feed table, having the vertical pairs of guide rods 7 and rollers 8.

The cell roll boxes are secured together by means of U-shaped clamps 48 and the ends of the units are insulated from each other by means of panels 49 forming gaskets between the same. Each panel is provided with a central reinforcing plate 50 of steel to prevent warping which is covered with insulating material such as rubber or the like. These panels 49 have a vertical central slot formed therein as at 51 for the sheet to pass through. The panels also have attached thereto adjacent to the slots porcelain guides 52 for guiding the sheet into or out of the different units and the input and output sealing flaps 53 and 54 respectively.

The plating cells are provided with a pipe 55 adapted to supply electrolyte thereto and pipes 56 for receiving the overflow of the electrolyte from the plating cells and conveying it to the launder 4, and thence to a sump. The anodic cell 12 is also provided with a pipe 57 for supplying a pickling bath thereto and overflow pipes 58 for conveying the pickling bath to the launder 5.

In the anodic cell 32 the same electrolyte may be used as that for the plating cells and will receive its supply in a similar manner through the pipe 59 and the overflow will be received by pipes 60 and returned to the launder 4.

As indicated in Figure 1 the contact and squeegee rolls are rotated by means of a motor 61 and driving mechanism which is more clearly illustrated and described in my copending application Serial No. 323,300.

When necessary to cool the cell wall electrodes the cells may be water jacketed as shown in cell 12.

This is particularly desirable when the cell walls are used as cathodes in an anodic treatment of the work since in this case a large portion of the ohmic heating of the solution occurs in the hydrogen gas layer at the cathode. To remove this heat with maximum efficiency the cell may be provided with a water jacket 62 formed by having a plate 63 secured to the lining 64 by means of studs 65. The jackets thus formed are supplied with inlet and outlet pipes 66 and 67 respectively.

In order to secure substantially uniform electrolytic action on each side of the work as it passes through the cells it is necessary to hold the work in uniform spaced relation with the electrodes or sides of the cells. This is accomplished by securing a plurality of porcelain guides 68 of frusto-conical shape to the inner sides of the lead lining of the cells. Each guide on one side of the cell is in transverse alignment with the opposite side of the cell. These frusto-conical guides have their inner surfaces far enough apart to allow the sheet 6 to pass freely between them and are so disposed that the shielding effect will be as uniformly distributed as possible.

Referring to Figure 1 it will be noted that the motor generator 69 furnishes the current through the bus bars 70 and 71 and terminal connections to the contact rolls and plating cells on one side

of the apparatus, the negative side of the circuit extending to the contact rolls, while the positive side of the circuit is connected to one side of the plating cells, and the motor generator 72 supplies the current through the bus bars 73 and 74 and terminal connections in a similar manner to the contact rolls and plating cells on the opposite side of the apparatus. With this system of connections and with opposite sides of the cells insulated from each other it is possible to vary the electrolytic effect on either side of the work by varying the current output of the two generators.

A more usual system of connections to a plurality of cells is to connect both sides of each cell to one generator, and, in case a plurality of generators are to be used to connect each generator to a cell or group of cells in succession through the apparatus.

The polarity for the anodic cells 12 and 32 is reversed to that of the plating cells. In these two cells the positive side of the circuit 35 from the motor generator 75 is connected to both pairs of contact rolls 10 and 33, while the negative side 36 is connected to both sides of each cell. In this manner of connecting up the circuit the work or sheet 6 will be the anode and the lead lining of the cell the cathode.

In many cases, a metallic coating deposited electrolytically upon the sheet or strip is of dull appearance and of relatively rough texture. It may also be discolored by oxidation after emerging from the plating bath or by chemical attack of the electrolyte upon it. In addition to washing the work at the exit end of the plating apparatus as elsewhere described, I apply one or more electro-chemical treatments to the work in a cell or cells located adjacent to the plating cells at the exit end of the apparatus by reversing the polarity in which the electro-deposited coating is acted upon anodically in the plating electrolyte as indicated in Figure 1, or I may use a separate electrolyte and electric circuit connections for the purpose for brightening or smoothing the surface of the coating by partially deplating the work.

Although I have shown and described my invention in considerable detail, I do not wish to be limited to the exact and specific details shown and described, but may use such substitutions, modifications or equivalents thereof as are embraced within the scope of my invention or as pointed out in the claims.

Having thus described my invention, what I claim as new and desire to secure by Letters Patent is:

1. The method of coating and polishing a sheet of ferrous metal with zinc by electrodeposition in a continuously progressing operation, which comprises subjecting the sheet as an anode to the action of an electric current in the presence of an electrolyte to clean the sheet, then subjecting the sheet as a cathode to the action of an electric current in a cell containing an electrolyte consisting essentially of zinc sulphate and sulphuric acid dissolved in water having an electric current connection on each side of the cell to plate the sheet, and finally polishing the zinc coating by subjecting the sheet without access to the air after the plating operation while still submerged as an anode to the action of an electric current in the presence of the same electrolyte used for zinc plating to slightly deplate the coating on the plated sheet.

2. The method of coating and polishing a sheet of ferrous metal with zinc by electrodeposition in a continuously progressing operation, which con-

sists in subjecting the sheet as an anode to the action of an electric current in the presence of an electrolyte to clean the sheet, subjecting the sheet continuously submerged as a cathode to the action of an electric current in a plurality of cells containing an electrolyte consisting essentially of zinc sulphate and sulphuric acid dissolved in water in succession each having an individual electric current connection on each side of the cell to plate the sheet, and finally polishing the 10 zinc coating by subjecting the sheet as an anode without access to the air after the plating operation to the action of an electric current in the presence of the same electrolyte used for zinc plating to slightly deplate the coating on the 15 plated sheet.

3. The method of coating and polishing a sheet of metal with zinc by electrodeposition in a continuously progressing operation, which comprises continuously subjecting portions of the sheet as 20 an anode to the action of an electric current in the presence of an electrolyte to clean the sheet, then subjecting the clean portions of the sheet as a cathode to the action of an electric current in the presence of an electrolyte consisting of an 25 aqueous solution of zinc sulphate and sulphuric acid for zinc plating, and finally polishing the zinc coating by again reversing the polarity of the sheet and subjecting the plated portions of the sheet as an anode while still submerged to an electric current in the same electrolyte used for zinc plating to slightly deplate the coating on the sheet.

4. The method of polishing a zinc coating which has been produced by electrodeposition on 30 a sheet of metal, consisting of subjecting the zinc plated sheet immediately after the plating operation and while still submerged in the electrolyte as an anode to the action of an electric current in the presence of the same electrolyte consisting of an aqueous solution of zinc sulphate and sulphuric acid similar to that used in coating without access to the air between the two operations to slightly deplate the coating on the plated 35 sheet.

5. The method of coating and polishing a sheet of metal by electrodeposition progressively by advancing the sheet through a plurality of cells each containing an electrolyte and having an electric circuit, which consists in first subjecting the sheet as an anode in a bath to clean the sheet, then conducting the sheet through a plurality of cells continuously submerged in an electrolyte consisting of an aqueous solution of zinc sulphate and sulphuric acid as a cathode to plate the sheet, and finally polishing the zinc coating by passing the sheet while still submerged through the same electrolyte used for zinc plating as an anode to slightly deplate the coating on the sheet.

6. The method of coating and treating a sheet of metal progressively by electrodeposition, which consists in advancing the sheet through a pickling bath as an anode to clean the sheet, thence into a plating bath consisting of an aqueous solution of zinc sulphate and sulphuric acid in a cell as a cathode to plate the sheet, and finally polishing the zinc coating while still submerged by advancing the plated sheet into a cell communicating with the plating cell containing the same electrolyte used for zinc plating as an anode to slightly deplate the surface of the coating on the sheet.

7. The method of coating and treating a sheet of metal or the like progressively by electrodeposition, which comprises subjecting the sheet as an anode to the action of an electric current in the presence of an electrolyte to clean the surface of the sheet, then subjecting the sheet as a cathode to the action of an electric current in the presence of a plating bath consisting of an aqueous solution of zinc sulphate and sulphuric acid to plate the sheet, and finally polishing the zinc coating while still submerged by again reversing the polarity of the sheet and subjecting the plated sheet as an anode to an electric current in a cell communicating with the plating cell to a portion of the same plating bath used for zinc plating to slightly deplate the coating on the sheet.

45 CLEMSON H. WARD.